

# UNITED STATES PATENT OFFICE.

AUGUSTUS ROSENBERG, OF LONDON, ENGLAND.

## PROCESS OF AND MEANS FOR DEPOSITING METALS.

970,852.

Specification of Letters Patent. Patented Sept. 20, 1910.

No Drawing. Original application filed March 16, 1909, Serial No. 483,748. Divided and this application filed August 2, 1910. Serial No. 575,115.

*To all whom it may concern:*

Be it known that I, AUGUSTUS ROSENBERG, a subject of the King of Great Britain, and resident of London, W. C., England, have 5 invented a Process of and Means for Depositing Metals, of which the following is a specification.

This application is a division of my application for patent for the same invention, 10 filed March 16, 1909, Serial No. 483,748.

This invention relates to the art of coating or plating electrically conductive surfaces with metals and to that particular method in which the article is coated by the 15 frictional application of a powder to its surface. My invention differs however from such method inasmuch as it is based on the employment of a novel mixture of ingredients containing all that is necessary, when 20 the mixture is brought into contact with water, to set up electrolytic action so that actual electrodeposition of the metal is brought about by electrolytic action notwithstanding that no external source of 25 current is employed. The process may be conveniently carried into effect by dipping a wet rag into the mixture so as to cause it to take up or become loaded with a sufficient quantity of the mixture and then rubbing 30 the mixture adhering to the rag onto the surface of the article to be coated and repeating the operation as often as necessary to obtain the desired result.

One object of my invention is to provide 35 a mixture whereby the electrolytic deposition may be carried out without the exercise of any skill, and in an efficient and economical manner, so as to permit the wide and convenient use of this powder for domestic or household purposes.

Another object of the invention is to provide 40 a mixture by means of which a firmly adherent and substantial deposit may be produced in the manner described.

A further object of my invention is to provide 45 a mixture of the kind referred to which may be kept indefinitely without losing its necessary qualities.

Other objects of my invention will be apparent 50 from the following description and to these and the foregoing ends my invention consists in the particular combination of ingredients all in powdery form, for obtaining the deposition of metals and the use thereof

as hereinafter specifically described and defined in the appended claims.

A further object of my invention consists in the employment, in combination with the metal to be deposited, of a metal in its elementary state, electropositive with respect to 60 the surface to be coated, and a substance which is capable of producing an aqueous electrolyte when brought into contact with water. In use, the substances in suspension (or in solution) in the electrolyte, as the 65 case may be, set up electrolytic action which brings about the deposition of metal upon the surface to be coated. The electropositive metal may in some cases be the metal to be deposited.

Another important feature of my invention consists in the combination with the ingredients of inert substances (either of mineral or organic nature) which by their presence will prevent premature interaction of 75 the ingredients which would otherwise take place or their chemical change previous to use.

A further feature of my invention consists in the use in the electroplating mixture 80 of a substance or substances which acts (or acts) either chemically or mechanically to impart a polish to the surface of the metal deposited.

As an example of a mixture prepared in 85 accordance with my invention I will give the formula of a mixture suitable for use in plating metals such as iron or copper with zinc. This formula is as follows:

|                           |           |     |
|---------------------------|-----------|-----|
| Zinc dust (commercial) -- | 45 parts. | 90  |
| Ammonium sulfate -----    | 15 "      |     |
| Magnesium -----           | 3 "       |     |
| Chalk -----               | 30 "      |     |
| Talc powder -----         | 7 "       | 95  |
|                           |           | 100 |

In this example the electropositive metal above referred to is the magnesium which is particularly adapted for the purpose as it is 100 electropositive with respect to all of the common metals generally used for plating. It is to be noted in general that in every case where the metal to be deposited is not, in itself, employed as the electropositive element hereinafter referred to, the metal which is so employed as electropositive element must not only be electropositive with

respect to the metal to be deposited but also to the surface to be plated.

The ammonium sulfate in the above formula constitutes, when moistened with 5 water, the electrolyte. In this connection it may be noted that the use of an ammoniacal salt as an electrolyte is particularly recommended when the surface to be plated is greasy, as the alkaline solution of 10 the ammonia gas liberated in the reaction dissolves the grease and thus facilitates the plating operation.

The commercial zinc of the formula above given contains impurities, including the zinc 15 oxid, but it is nevertheless quite suitable for use, as the impurities are not such as to substantially interfere with the necessary reactions, while the oxid is dissolved and the zinc therein deposited the same as in the 20 case of the elemental zinc. In this connection it may be noted that in general the oxids of the metals to be deposited may be employed in place of these metals in elemental form, where an electropositive metal is also 25 employed, and in the succeeding claims, where I have specified a metal in "elemental" form as the metal to be deposited, I do not mean to exclude the oxid of such metal.

30 The talc powder in the above formula has the function of preventing the ammonium sulfate from acting upon the other ingredients in consequence of the absorption of moisture from the atmosphere, and the use 35 of this or an equivalent substance is an important feature of the invention, since it permits the mixture to be stored or to be exposed to the atmosphere for lengthy periods without substantial deterioration.

40 The chalk of the formula acts as a diluent or filling and retards the action of the elements of the compound on each other, thereby affording the necessary time for the electrolytic action to occur in the best manner. The chalk is also useful, as it insures 45 an alkaline reaction in the electrolyte. The chalk has a further mechanical function which will be referred to later.

In the above-described operation the chalk, 50 in addition to the functions specifically described, acts as a mechanical polishing agent, so that the frictional application of the mixture results; first, in the cleansing and polishing of the conductive surface; second, in 55 the deposition of the zinc, and third, in polishing the newly deposited zinc.

In addition to the use of mechanical polishing agents, I may make use of agents having a chemical effect resulting in a polished surface on the deposited metal. For 60 this purpose I have found carbohydrates, such as sugar, dextrin, and gum to be effective when employed in a mixture in which the electrolyte is a sulfate or a double salt 65 containing the radicle  $\text{SO}_4$ , the later prob-

ably forming with the carbon of the carbohydrates, carbon disulfid, a substance which is well known to have a polishing or brightening effect upon electrically deposited metal.

The friction employed in applying my electro-plating mixture is useful in several ways. It acts, first, to assist the cleaning of the surface to be plated. It assists the chemical and electrical actions by bringing 70 the elements of the mixture in close contact and by mechanically depolarizing the metallic elements of the electric couples by which the electric current is generated. Finally it acts, as before pointed out, to polish the deposited metal.

While the talc powder acts as above pointed out to prevent the absorption of moisture from the atmosphere and thus to prevent premature chemical action between the ingredients of the mixture, I find it useful, particularly where a strongly electropositive metal, such as magnesium, is employed, to prevent oxidation and protect such metal absolutely from contact with the corrosive 85 electrolytic salt, and to this end I have devised the expedient of coating the particles of the electropositive metal with an inert substance preferably of waterproof character, for which purpose I find organic substances, such as waxes and resins to be suitable. The most convenient way in which 90 to coat the particles is to moisten them with a solution of wax or resin in gasoline or other volatile solvent, and then dry out the 100 solvent, after which the coated metal is mixed with the other ingredients of the mixture. When the mixture is used the friction employed in the application quickly causes the removal of the coating material 105 and the exposure of the metal to the electrolyte. The coating of the electropositive metal has the further advantage (where the metal to be deposited is present in elemental form, as in the formula hereinbefore given 110 for zinc-plating) that it prevents chemical action upon the electropositive metal upon the first wetting of the mixture, and this affords opportunity for the metal in suspension to be deposited.

In addition to the ingredients hereinbefore mentioned, it may sometimes be desirable to add certain acid substances, such as boracic acid, or alkalies, such as sodium carbonate, in order to give the composition 120 either an acid reaction or an alkaline reaction, as may be desirable under circumstances well known to those skilled in the art of electroplating.

My invention is applicable for depositing 125 almost any metal upon itself, for example, zinc upon zinc, or upon any other metal generally used in the art of electroplating, and it will be understood that the several ingredients hereinabove referred to may be 130

an electrode or other object is suspended and placed in a tank containing the electrolyte, a metal electropositive with respect to said surface and in elemental and comminuted form, is used in proportions widely varying from those given in the preceding formula, and that the use of some of them is optional and is governed by the widely varying purposes for which my invention may be used.

In the application of the mixture in the manner described, the electropositive metal constitutes the anode and the object to be coated the cathode and both being in suspension in the electrolyte, current is generated. Owing to the comminuted state of the electropositive metal, innumerable small contacts with the cathode surface are made and the particles of electropositive metal act as so many minute anodes, each setting up local circulations of electric current. The circuits are so excessively small, so exceedingly near together and so numerous that they cannot be separately observed, but each causes a deposit of the metal to be deposited upon the cathode surface. Owing to the number of small currents generated these, as they leave the liquid, deposit a film of the metal to be deposited over the surface to be coated.

The foregoing description of the manner of carrying out my invention is for the purpose of illustration only and is not intended to be exclusive.

30 It is also obvious that many modifications and changes may be made in my invention without departing from the spirit of the same, and I do not desire to limit myself to the particular features described, but

35 What I claim and desire to secure by Letters Patent is:—

1. The method of electroplating which consists in the frictional application to an electrically conductive surface, in the presence of an electrolyte containing in suspension the metal to be deposited, of a second metal electropositive with respect to both said surface and said metal in suspension, said electropositive metal being in elemental and comminuted form.

2. The method of electroplating which consists in the application to an electrically conductive surface, in the presence of an electrolyte, of the metal to be deposited together with a polishing agent.

3. The method of electroplating which consists in the frictional application, to an electrically conductive surface, in the presence of an electrolyte, of the metal to be deposited, together with a mechanical polishing agent.

4. The method of electroplating which consists in the frictional application, to an electrically conductive surface, of a mixture comprising an electrolyte, a carbohydrate, and a metal electropositive with respect to said surface and in elemental and comminuted form.

5. The method of electroplating which consists in the frictional application, to an

electrically conductive surface, in the presence of an electrolyte and a solid diluent, of a metal electropositive with respect to said surface and in elemental and comminuted form.

6. The method of electroplating which consists in the application, to an electrically conductive surface, in the presence of a solid diluent and of an electrolyte containing in suspension the metal to be deposited, of a second metal electropositive with respect to both said surface and the metal in suspension, said electropositive metal being in elemental and comminuted form.

7. The method of electroplating which consists in the application, to an electrically conductive surface, of a mixture comprising comminuted, elemental magnesium, and an electrolyte having in suspension the metal to be deposited.

8. The method of electroplating which consists in the frictional application, to an electrically conductive surface, in the presence of an electrolyte holding in suspension the metal to be deposited, of comminuted elemental magnesium.

9. The method of manufacturing an electroplating mixture which consists in coating electropositive metal particles in the elementary and comminuted form with a solution of protective material, drying said particles, and mixing them with the metal to be deposited.

10. The method of manufacturing an electroplating mixture which consists in coating metal particles with a protective material, and mixing the coated particles with a dry pulverulent material capable of forming an electrolyte.

11. The method of electroplating, consisting in the frictional application to a conductive surface in the presence of moisture, of a mixture of pulverulent materials including the metal to be deposited, an electropositive metal and a substance capable of yielding, in conjunction with moisture, an aqueous electrolyte.

12. The method of electroplating, consisting in the frictional application to a conductive surface in the presence of moisture, of a mixture containing pulverulent materials, including the metal to be deposited, an electropositive metal present in the elementary state and a substance capable of yielding, in conjunction with moisture, and an aqueous electrolyte.

13. As a new article of manufacture for depositing a metal upon a conductive surface, a mixture of pulverulent materials including the metal to be deposited, an electropositive metal, and a substance capable of yielding, in conjunction with moisture, an aqueous electrolyte.

14. As a new article of manufacture for depositing a metal on a conductive surface,

a mixture of pulverulent materials including the metal to be deposited in its elementary form, an electropositive metal, and a substance capable of yielding, in conjunction with moisture, an aqueous electrolyte.

15. As a new article of manufacture for depositing a metal upon a conductive surface, a mixture of pulverulent materials including the metal to be deposited, an electro-

10 positive metal, and a salt.

16. As a new article of manufacture for depositing a metal upon a conductive surface, a mixture of pulverulent materials including the metal to be deposited, an elec-

15 tropositive metal, a salt, and a substance capable of preventing the absorption of moisture.

17. As a new article of manufacture for

depositing a metal upon a conductive surface, a mixture of pulverulent material including the metal to be deposited in elementary form, an electropositive metal, and a metallic salt.

18. As a new article of manufacture for depositing a metal upon a conductive surface, a mixture of pulverulent material including the metal to be deposited in elementary form, an electropositive metal, a metallic salt, and a substance capable of preventing the absorption of moisture by the said salt.

AUGUSTUS ROSENBERG.

Witnesses:

H. D. JAMESON,  
R. WILLIAMS.